

Sept. 9, 1952

F. H. MASON

2,609,598

METHOD OF FORMING A COMPOSITE STRUCTURE  
COMPRISING A CHROME-CONTAINING MEMBER  
Filed Sept. 27, 1947



INVENTOR.

Frederick H. Mason

BY

Harnes and Harris  
ATTORNEYS.

## UNITED STATES PATENT OFFICE

2,609,598

METHOD OF FORMING A COMPOSITE  
STRUCTURE COMPRISING A CHROME-  
CONTAINING MEMBERFrederick H. Mason, Detroit, Mich., assignor to  
Chrysler Corporation, Highland Park, Mich., a  
corporation of Delaware

Application September 27, 1947, Serial No. 776,485

2 Claims. (Cl. 29—378)

1

This application relates to a method of joining parts by means of a metallic bond. More specifically, it relates to a bonding process involving applying a preliminary coating to one of a plurality of objects to be joined, which object would be damaged by the use of flux otherwise required in the bonding process but for the use of the coating.

The process of this invention may be applied to the bonding of parts containing a percentage of chromium sufficient to form a bond-resisting oxide upon being heated for bonding. If the aforesaid parts are thin-walled tubes, for example, the flux required to prevent the formation of chromium oxide will eat through the thin tube walls, unless resort is had, not to the ordinary brazing atmosphere, but to one that is very free of oxide-forming components such as oxygen and especially moisture and thus is very expensive.

The thin-walled tubes may be bonded to other parts to form a regenerator or heat exchanger for recovering waste heat from a gas turbine and applying it to air going to burners supplying hot gases for the aforesaid gas turbine.

In the drawings:

Fig. 1 shows a plate and tube positioned in an opening in the plate;

Fig. 2 shows the plate and tube of Fig. 1 after the tube has been expanded;

Fig. 3 shows the plate and tube after they have been bonded to one another; and

Fig. 4 shows an alternate process for joining the tube and plate.

Reference character 10 designates a nickel plate having on one side a chromium coating 11 and on the other side a copper coating 12. The plate 10 has an opening 13 in which is positioned a chromium-containing tube 14, which may have, for example, such compositions as 13% chromium and the balance nickel; 18% chromium, 8% nickel, a small amount of columbium, and the balance iron; and 20% chromium, 65% cobalt, and the balance tungsten and nickel. The coating of tube 14 with nickel plating 16 is carried out when the surface of the tube is free of oxide and foreign matter and at the plating temperatures involved there is little, if any, tendency for chromium oxides to form from the chromium content of the tube. The present improvement, however, is most advantageously carried out when the tube has sufficient percentage of chromium to form a bond-resisting oxide on heating subsequently to plating to the relatively higher temperatures necessary for bonding. About 5% chromium is sufficient for forming the above bond-resisting oxide. The nickel coating may be applied to a tube of pure chromium, although it is more advantageously used when the tube contains another metal permitting the nickel coating to alloy by diffusion with the tube more readily than when the tube contains only chromium.

2

The tube 14 has an external circumferential bulge 15 adjacent the chromium-coated side of the plate 10 and a nickel coating 16 extending from the bulge 15 extending perhaps as far as the very end of the tube 14. The portion of the tube 14 to the left of the copper-coated side of the plate 10 is expanded, as indicated in Fig. 2, by a suitable tool, not shown, and so a very small annular opening 11a is formed between the nickel coating 16 at the start of the expansion and the edge of the copper plating 12 at the hole 13.

Now the plate 10 and tube 14 are placed in a brazing atmosphere and subjected to a brazing process involving at least six hours at 1500° F. and above, and a top temperature of 2100° F. The time and temperature are sufficient for the copper coating 12 to melt and to be drawn by capillary action through the annular space 16a into the clearance space shown in Figs. 1 and 2 between the nickel coating 16 and the tube 14 and the plate opening 13 and to alloy with the nickel of the plate 10 and with the nickel coating 16 on the tube 14. The copper-nickel alloy forms a good heat resistant bond sufficient for the purposes to which the tube and plate are to be put, as will be described later. The nickel coating 16 does not completely alloy with the tube 14, but the alloying is sufficient to insure good bond between the coating and the tube thereby making the copper-nickel bond effectively seal the tube 13 to the plate 10.

If it is not feasible to extend the length of the present process to six hours above 1500° F. as previously mentioned, the tube and its coating may be subjected to a suitable heating process before assembly of the tube and plate to effect a sufficient alloying of the coating and tube by diffusion for a good joint between the coating and the tube. Alternately, such a heating operation may be carried on after the brazing has been effected.

The bulge 15 may be formed before or after the coating 16 is applied to the tube 14. It will be convenient to apply the coatings 11 and 12 to the plate 10 before the hole 13 is formed therein. The various coatings 11, 12, and 16 may be applied by the process of electrodeposition. Special care must be taken in the case of the nickel coating 16 on the tube 14 to insure that all oxides have been removed from the portion of the tube to be coated, because any oxide left beneath the coating 16 may blister during the present process and thereby interfere with the strength of the metallic bond formed.

As shown in Fig. 3, some of the copper coating 12 remains on the plate 10, having alloyed with the plate, because the present process may involve an appreciable time above 1500° F., at which alloying by diffusion takes place at an appreciable rate, and below 1960° F., the temperature at which copper melts and will run into the space between

the tube coating 16 and the hole 13. The extended heating and brazing process also causes the chromium coating 11 to alloy by diffusion to some extent with the nickel plate 10.

The nickel coating 16 has been applied to the tube 14 as a preliminary step to the present operation, because the relatively high chromium content of the tube 14 would cause the present heat to produce bond-resisting chromium oxide on the tube 14, which could be avoided only with the use of a very expensive atmosphere that is free of oxygen-forming impurities, particularly moisture or by the use of a flux which has a tendency to eat through the wall of the tube 14, which in a desired example is only about .005" in thickness.

When the thickness of the tube 16 is about .005" as above mentioned, the nickel coating 16 may be .003" to .005", the copper coating 12, .015", and the chromium coating 11, .002". The difference in diameter between the coated portion of the tube 14 and the hole 13 may vary from .001" to .01". In any event, the tight fit employed between steel parts about to be brazed with copper is not used with the nickel-coated tube 14 and the nickel plate 10, because copper flows less readily on nickel than on steel.

In the alternate process of Fig. 4 the end of the tube 14 is left unexpanded and a copper ring 17 is substituted for the copper coating 12. When the parts of Fig. 4 are heated, the copper ring 17 is melted and drawn into the space between plate opening 13 and the tube coating 16 and alloys therewith, as previously described, with respect to Figs. 1, 2, and 3. The advantage of the construction of Fig. 3 is that the expanded portions of the tube 14 at both sides of the plate 10 relieve the copper-nickel bond of stresses due to limited longitudinal movement of the tube with respect to the plate.

Broadly speaking, the nickel coating 16 is applied to the tube 14, because the tube contains chromium in a percentage sufficient to form a bond-resisting oxide, which is about 5%. No coating need be applied to the hole 13 in the plate 10, because the plate contains less than the 5% chromium leading to the formation of the bond-resisting oxide, and in actual fact, no chromium.

The joint construction described with reference to Figs. 1 to 4 inclusive, may be used in a regenerator or heat exchanger for recovering waste heat from the exhaust to the gas turbine and applying the waste heat to air fed to burners supplying gases for the gas turbine. In the regenerator the plate 10 may be a bulk head or sheet to which a plurality of parallel tubes 14 are bonded and attached, and there is a bulk head on each end of the tubes. Hot gases coming from the turbine come into contact with the exterior of the tubes 14 between the plates or bulk heads 10 and air on its way to the burners supplying the turbine is fed through the tubes 14. The chromium coating 11 on the plate 10 provides good resistance to the hot gases coming from the turbine, especially if they contain sulphur.

I claim:

1. A method of bonding comprising providing a nickel plate having a hole and a coating of copper on one side around the hole and a tube containing nickel and chromium with an external bulge greater in external diameter than the hole in the plate and spaced from one end of the tube a distance greater than the thickness of the plate and an external coating of nickel extending from the bulge toward the said one end of the tube, placing

the tube in the hole in the plate so as to make a portion of the tube adjacent the said one end thereof to extend beyond the copper-coated side of the plate, the tube bulge and the other side of the plate to be juxtaposed, and the plate hole directly to surround a nickel-coated region of the tube, expanding the said tube portion beyond the copper-coated side of the plate to make the outer diameter of the said tube portion greater than the diameter of the plate hole and the said tube portion to form with the copper-coated side of the plate a very small annular opening leading to the space between the plate hole and the nickel coating on the tube, heating the plate and the tube to a temperature above 1500° F. at which the nickel coating on the tube alloys with the tube, and maintaining at a temperature above 1500° for a sufficient time for the nickel coating on the tube to alloy with the chromium-containing tube without the chromium penetrating through the nickel coating in substantial quantities to the external surface of the latter and at a temperature up to 2100° F. to cause the copper coating on the plate to be drawn through the aforesaid annular opening and to alloy with the plate hole and the nickel coating on the tube.

2. A method of bonding a first part having a surface containing nickel and more than about 5% chromium to a second part having a surface containing nickel and less than about 5% chromium, said method comprising coating the surface of the first part with nickel, juxtaposing the parts so as to bring the surface of the second part in closely spaced relation to the nickel coating on the surface of the first part, applying heat to the juxtaposed parts in the presence of a copper bonding metal for the ultimate bonding of the same together, to a temperature above 1500° F. at which the nickel coating alloys with the first part, and maintaining the parts at a temperature above 1500° F. for a sufficient time for the nickel coating on the first part to alloy with the chromium-containing first part without the chromium thereof penetrating through the nickel coating in substantial quantities to the external surface of the latter and at a temperature up to 2100° F. for causing the copper metal to melt in order to flow between the nickel coating and the surface on the second member and alloy therewith.

FREDERICK H. MASON.

#### REFERENCES CITED

The following references are of record in the file of this patent:

#### UNITED STATES PATENTS

| Number    | Name       | Date          |
|-----------|------------|---------------|
| 1,250,881 | Hodges     | Dec. 18, 1917 |
| 1,804,237 | Steenstrup | May 5, 1931   |
| 2,117,106 | Silliman   | May 10, 1938  |
| 2,123,384 | Silliman   | July 12, 1938 |
| 2,197,039 | Gottlieb   | Apr. 16, 1940 |
| 2,269,523 | Deutsch    | Jan. 13, 1942 |
| 2,364,109 | Taylor     | Dec. 5, 1944  |
| 2,390,452 | Mudge      | Dec. 4, 1945  |
| 2,446,890 | Gilbertson | Apr. 12, 1949 |

#### FOREIGN PATENTS

| Number  | Country       | Date          |
|---------|---------------|---------------|
| 309,032 | Great Britain | Oct. 24, 1929 |
| 547,755 | Great Britain | Sept. 2, 1942 |

#### OTHER REFERENCES

Steel Mag., July 21, 1947, Furnace Brazing, pp. 103, 104, 106, 124 and 127.

Methods for Placing Brazing Materials, and Vent Locations, Prod. Eng., July 1947, p. 127.